

## UNITED STATES PATENT OFFICE

2,196,796

PROCESS FOR IMPROVING DRYING  
PROPERTIES OF OILSTheodore S. Hodgins, Royal Oak, Mich., assignor  
to Reichhold Chemicals, Inc., formerly Beck,  
Koller & Company, Inc., Detroit, Mich.No Drawing. Application July 17, 1939,  
Serial No. 285,001

4 Claims. (Cl. 260—423)

In common with the disclosure of my Patent No. 2,133,894 dated October 18, 1938, the present invention relates broadly to a process for improving the drying properties of naturally occurring 5 anti-oxidants.

According to the process claimed in said patent it was shown that the drying properties of such oils could be improved by treating the oils, preferably at substantially room temperature, with 10 the use of a relatively strong inorganic oxidizing agent, provided the pH value of the solution was maintained close to the neutral point while avoiding exact neutrality, by the use of either an alkaline or an acid reagent in certain specified 15 quantities with respect to the weight of the oil. The optimum range in the case of the alkali was found to be .013-.050 part by weight of alkali to 100 parts by weight of the oil, and in the case of the acid reagent the range was .025-.050 part by 20 weight of acid to 100 parts by weight of the oil being treated.

In my application Serial No. 240,858 filed November 16, 1938, now Patent No. 2,167,206 dated July 25, 1939, it was shown that similar results 25 could be obtained by the use of an organic oxidizing agent such as benzoyl peroxide, and properly controlling the pH value of the solution by the use of an acid or alkaline reagent in the proportion of approximately 1-5% by weight of the oil 30 being treated.

The present application is specifically directed to the improving of oils using a definite quantity of a reagent which serves the dual function of an oxidizing agent and of a reagent for controlling 35 the pH value of the solution. I have found that concentrated nitric acid fulfills this double function. The quantity of this acid employed may vary substantially within the range of .025-0.50% by weight of the oil, particularly good results 40 being obtainable when concentrated nitric acid in the proportion of about 0.20% by weight is employed.

Various types of oils containing naturally occurring anti-oxidants may be improved as to 45 their drying properties by treatment in accordance with the present process, among which may be mentioned by way of example linseed oil, soya bean oil, sunflower oil, perilla oil, rapeseed oil and oiticica oil.

50 The length of time required for treating these oils is determined by the first measurable increase in refractive index or by a corresponding decrease in iodine number. The method of treatment of an oil comprises treating the oil preferably at 55 room temperature with a small quantity of nitric

acid within the limited range referred to above. The process effectively removes the anti-oxidants (such as lecithin and cephalin) which are naturally occurring in these oils. The sludge containing the anti-oxidants and spent reagents 5 may be separated from the refined oil in any suitable manner, such as by filtering, centrifuging, or the like, depending on the nature of the treating solution.

I am aware that previous attempts have been 10 made to improve the drying properties of oils by partially oxidizing the same, particularly by passing air or other oxidizing gas through the body of the oil. My invention is not concerned with this 15 type of oxidation. In such prior processes the oxidation has taken place within the oil itself whereas according to my process only the anti-oxidants are eliminated, the oil being unoxidized. Also in such previous treatments temperatures above 20 room temperature have been considered necessary 20 whereas my process may be carried on to best advantage at substantially room temperature.

It has also been proposed to treat various oils with chemical reagents such as acids, alkalies and salts for the purpose of improving their qualities, 25 as for example for removing odors or bleaching the same, but to my knowledge no successful process has been carried out at room temperature wherein the anti-oxidants are removed by treatment at room temperature employing a small pre- 30 determined quantity of an oxidizing agent which also serves to control the acidity of the solution within definite limits.

The invention will be more readily understood 35 by reference to the following specific example.

## Example

## Parts by weight

|                          |           |
|--------------------------|-----------|
| Sunflower oil            | 100       |
| Concentrated nitric acid | 0.2       |
| Water (not constant)     | 1.0 to 10 |

The oil is preferably treated for one-half hour to two hours and may be mechanically agitated either by means of a stirrer or by blowing filtered air or an inert gas through the material, it being 45 understood that the air or gas employed functions solely as an agitating means and does not in any way enter into the reaction. The time may be varied according to the particular conditions employed, the exact time in any particular instance 50 being determined by a refractive index curve such as shown in Fig. 2 of my prior Patent No. 2,133,894. The complete destruction of anti-oxidants is determined when the refractive index first begins to increase. The treatment may be 55

carried out at substantially room temperature and the decomposed impurities filtered or otherwise separated out. The resultant oil is found to be much improved in drying properties as compared to the original oil and has a slightly lighter color.

While sunflower oil is specifically referred to in the above example, it will be understood that various other oils containing anti-oxidants may be substituted with similarly improved drying properties, in the final product.

I claim:

1. A process for improving the drying quality of raw oils containing naturally occurring anti-oxidants, which comprises removing the anti-oxidants by treating the oil at substantially room temperature with nitric acid, and maintaining the pH value of the materials undergoing treat-

ment only slightly acid throughout the treatment by confining the quantity of nitric acid employed substantially within the range of .025-.50% by weight of the oil being treated, continuing the treatment just until the refractive index begins to increase, then discontinuing the treatment and separating the treated oils from the other constituents.

2. A process as set forth in claim 1, wherein the quantity of nitric acid employed is approximately 10 0.20 by weight of the oil being treated.

3. A process as set forth in claim 1, wherein the oil treated is a member of a group consisting of linseed oil, soya bean oil, sunflower oil, perilla oil, rapeseed oil and oiticica oil.

4. A process as set forth in claim 1, wherein the oil treated is sunflower oil.

THEODORE S. HODGINS.